

Feb. 15, 1944.

L. S. FRYER

2,341,842

## METHOD OF MANUFACTURING STAPLE FIBER

Filed April 11, 1941



## Inventor

LOUIS S. FRYER

Charles Herrstrom  
Attorney

## UNITED STATES PATENT OFFICE

2,341,842

## METHOD OF MANUFACTURING STAPLE FIBER

Louis S. Fryer, Cleveland, Ohio, assignor to Industrial Rayon Corporation, Cleveland, Ohio, a corporation of Delaware

Application April 11, 1941, Serial No. 388,124

9 Claims. (Cl. 18—54)

This invention relates to a method of manufacturing staple fiber adapted to be formed into a novel yarn. Among other things, the invention involves simultaneously producing a plurality of multiple filament thread bundles possessing diverse physical characteristics; reducing the thread bundles, preferably loosely aggregated, to fibers of staple length; drying the resulting fibers; and finally blending them so that the dissimilar features of the component fibers cooperate to produce a novel effect. Yarns spun from fibers so produced possess characteristics virtually unobtainable by ordinary procedures.

Whereas according to conventional methods of mixing fibers of dissimilar characteristics it is extremely difficult to obtain a completely uniform blend, the present invention gives rise to a blend of an unusually high degree of uniformity.

This characteristic is largely due to the fact that considerable preliminary commingling of the elements of the finished product takes place prior to the actual blending operation. Being of artificial origin, several threads may, for instance, be spun simultaneously, different physical characteristics being introduced into the different threads in the course of the spinning operation. Thereafter, even if possessed of like characteristics following the spinning step, the several threads may be subjected to processing treatments capable of altering certain of them. In any event, the threads may be reduced to fibers of staple length by an operation which facilitates later blending, such operation substantially modifying the original relationship of the threads.

An attribute of the process is the facility with which the combination of the component threads may be varied to produce different products. The appearance of the finished product may be altered by simply controlling the number of threads or thread bundles of each physical characteristic being produced, thereby determining which one of various possible effects is to predominate. One of the important advantages of the invention is this possibility of controlling in the minutest degree the combinations of the constituents and, ultimately, the appearance of the finished product.

Another advantage of the invention is the fact that it lends itself to the precise reproduction of novelty yarns. By present methods, according to which fibers of staple length must be very carefully combined and blended in an attempt to produce a desired product, it is frequently impossible to arrive twice at the same result except by cut and try methods. Unlike processes here-

tofore employed, the invention makes it possible to reproduce products previously manufactured. In the practice of the present invention, nothing more is required than a knowledge of the number of thread bundles, together with their respective characteristics, which were originally employed to make the yarn or fabric to be reproduced.

In the description which follows, the invention will be explained with reference to the accompanying drawing. In such drawing, Figure 1 represents a side elevation of apparatus suitable for the production, processing and cutting of multiple filament artificial silk thread bundles into fibers of staple length which are blended to give a highly uniform product. Part of the apparatus shown in Figure 1 is broken away to reveal the details of the blending apparatus. Figure 2 is a plan of the apparatus illustrated in Figure 1.

Broadly speaking, the apparatus shown in Figures 1 and 2 is generally similar to but not identical with that shown, described and claimed in Kline et al, Patent 2,233,418. It consists for the most part of a frame structure providing two operating faces extending lengthwise of the apparatus as a whole each of which consists of two superposed processing units. Each processing unit includes, in addition to a coagulating trough, a series of thread-manipulating devices by means of which a multiple filament thread bundle is subjected to processing treatment. The thread bundles from the several processing units pass in sequence to means for aggregating them to form a large but preferably open thread bundle, means for reducing to fibers of staple length the large thread bundle so formed, a drying chamber, and finally picking and blending means.

For the sake of simplicity, the apparatus, although capable of being used in the manufacture of products of various kinds, will be described as employed in the manufacture of products made by the viscose process. In such case, viscose used for spinning purposes is supplied to the machine from suitable storage facilities (not shown) by means of supply pipes 5. Pumps 6, to which supply pipes 5 are connected, serve to force the viscose through pipes 7 into mass tubes 8. Through each mass tube 8 the viscose passes to the corresponding spinneret 9, by means of which it is extruded into a coagulating bath 10 in trough 11 to form a thread 13a comprising a plurality of fine filaments.

In each processing unit, several threads 13a, all of which are formed in like fashion by similar

spinnerets 9, pass through or over a gathering guide 14 by means of which they are combined to form thread bundle 13b. The latter proceeds from one to another of a series of thread-advancing thread store devices which may advantageously take the form of thread-advancing reels 15, 15a, 15b, 15c, 15d, etc., upon which various processing operations are performed upon the thread bundle. Such thread-advancing reels, which operate on the principle described in Knebusch Patent 2,210,914, will be referred to hereinafter simply as "reels."

Reels 15, 15a, 15b, 15c and 15d, five in number, provide for the storage of the thread bundle 13b during processing. Typical processing stages include a holding stage followed in turn by a stage involving treatment with dilute acid, a washing stage, a desulfurizing stage, and a second washing stage. Additional reels may, if desired, be provided for the storage of the thread while it is being subjected to bleaching, oiling, additional washing and other like operations, depending upon the character of the desired product.

The supporting structure on which are mounted the reels of each processing unit comprises a plurality of vertical supports 16 between which are disposed longitudinally extending horizontal members 17 and cross members 18. On horizontal frame members 17 are mounted reel bearing brackets 19 through which extend reel shafts 20. Reels 15, 15a, 15b, 15c, 15d, etc., are so arranged that the unsupported end of each is in opposite relation to the supported end of the succeeding reel, whereby bundle 13b is enabled to pass from one to another of the reels without interruption.

Each reel shaft 20 is provided with a gear 22 which meshes with a gear 23 mounted on longitudinally extending drive shaft 24, one such drive shaft 24 being provided for each processing unit. A power source such, for example, as motor 25, is disposed at one end of the assembly. It actuates one of the lowermost drive shafts 24 by means of chain drive 26. Power for driving shafts 24 of adjacent processing units may advantageously be transmitted thereto by means of sets of intermeshing spur gears 27, 28 and chain drive 29. Each processing unit is provided with suitable clutch means 30 to control its operation.

Associated with each of the reels other than reel 15 is a collecting trough 32. It comprises a top portion 33, vertically extending sides 34, and bottom portion 35. Mounted upon one of the sides 34 of collecting trough 32 adjacent the supported end of reel 15a is a lead-on guide 36 by means of which thread bundle 13b is led to the supported end of said reel from reel 15. On the opposite side 34 of collecting trough 32 and adjacent the unsupported end of reel 15a is located take-off guide 37 which is employed to direct bundle 13b from the unsupported end of reel 15a to lead-on guide 36 associated with the succeeding reel.

Processing liquids for use in the apparatus are kept in suitable reservoirs (not shown). The appropriate processing liquid is led from such reservoir to the proper processing stage by means of supply pipe 38 to which is connected a distributor 39 which showers the liquor upon thread bundle 13b. An amount of liquid preferably slightly in excess of that required for the actual processing of thread bundle 13b is furnished by supply pipes 38. The processing liquid following its application to thread bundle 13b by distributor 39 drips off into collecting trough 32 disposed below each reel. The spent liquor is drained there-

from by means of drain pipe 42 after which it is either rejected or returned to the reservoir for re-use.

On the completion of the required processing steps, the thread bundles 13b leave the last reels of their respective processing units, in this case reels 15d, after which they are more or less loosely aggregated by means of a guide 43 so as to form a large thread bundle 13c. The identity of the individual thread bundles 13b is preferably maintained in such large thread bundle in order to facilitate reduction of the filaments to fibers. A guide having separate slots for each thread bundle 13b; i. e., a comb guide, may conveniently be employed for this purpose; however, a combining guide giving rise to a consolidated rather than an open thread bundle may, if desired, be used instead. In the drawing, thread bundle 13c is of the latter type; i. e., loosely aggregated.

For the purpose of reducing it to fibers of staple length, the large thread bundle so formed is subjected to a cutting operation. The cutting apparatus employed to this end is similar to that shown, described and claimed in Jordan Patent 2,201,180. By means of this apparatus, thread bundle 13c may be cut into chips of predetermined length, such chips being in the preferred embodiment of the invention of relatively small cross-sectional area. If a consolidated rather than an open thread bundle were to be formed by guide 43, the chips would naturally be relatively large.

The cutting unit comprises a base 45 on which is mounted a cutter 46. After passing through squeeze rolls 44, thread bundle 13c enters a guide tube 47 into which a stream of air can be directed if required to facilitate threading-up operations. On leaving guide tube 47, thread bundle 13c enters another guide tube 48 which directs it to feed rolls 49. A second comb guide may, if desired, be placed between guide tube 48 and feed rolls 49; however, in the apparatus shown no guide is employed at this point. Immediately after leaving feed rolls 49 thread bundle 13c proceeds to cutter housing 50.

Chips 52, formed by the cutting operation, drop onto a conveyor belt 53a of wire mesh fabric which passes around a pulley 54 suspended from cutter base 45 by means of a bracket 55. Belt 50 53a is the first of a series of several belts disposed in dryer 56. By means of such belts, chips 52 pass through dryer 56 at a speed such that before reaching the discharge end of said dryer they are completely dried. At the discharge end 55 of conveyor belt 53c but within dryer 56 are disposed picking and blending means 57.

Chips 52, entering picking and blending means 57 by means of opening 58, come into immediate contact with feeder strippers 59, off which they are picked by breast cylinder 60. From breast cylinder 60 the worker rolls 62 and stripper rolls 63 pick off the fibers to continue the picking and blending process. Upon the completion of this operation, the blended fibers are discharged through outlet 64. Such fibers are ready to be spun into thread.

Apparatus of the type hereinabove described may be employed in the practice of the present invention by using two or more spinning solutions containing substances capable of developing diverse physical characteristics in the respective thread bundles 13b. It is equally possible in the case of the illustrated apparatus to spin a plurality of identical thread bundles 13b from the same spinning solution, subjecting them during

processing to the action of different treating media to the end that the thread bundles will have dissimilar physical characteristics. Thus the invention involves at least two general modes of operation, the result in each case being an improved final product.

The first-mentioned phase of the invention embraces the addition to the respective spinning solutions of delusterants, pigment colorants, vat dyestuffs or the like. Novel effects may be produced in the ultimate product by combining fibers of low luster spun from pigment-delustered solutions with bright fibers formed from ordinary lustrous spinning solutions. Similarly, a diversity of color combinations may be obtained by employing two or more spinning solutions to each of which has been added a different colorant. Obviously, these same factors may be employed simultaneously to give rise, for example, to combinations of colored lustrous fibers with uncolored delustered fibers, etc.

A unique result obtainable by this phase of the invention follows from the use of two spinning solutions each of which is colored with a different primary color. In such case, the finished staple fiber produced by combining component fibers of the two colors has the appearance of a single color. When, for example, two different spinning solutions respectively colored blue and yellow are employed, the color of the ultimate product is neither blue nor yellow but a distinct green. Despite the presence of the two primary colors in different fibers at the same time, the product as a whole has a monochromatic appearance.

The same result may be brought about by the use of any number of other primary colors which, when thoroughly blended, are virtually indistinguishable except upon close inspection, thus giving the product the appearance of a single secondary color.

Similarly, a color tint may be produced by combining fibers cut from colored thread bundles with fibers cut from thread bundles produced from uncolored spinning solutions. If, for instance, fibers spun from a spinning solution containing a blue colorant are combined in proper proportions with fibers spun from an uncolored solution, a shade of blue will be produced which is lighter in appearance than the original blue. In the same way, black fibers combined with fibers spun from uncolored spinning solutions will appear gray upon blending. However, under certain conditions, especially when colors of equal brilliance are used, blended staple fiber of relatively high filament titer may nevertheless present a heterochromatic appearance.

According to the second phase of the invention, two or more like thread bundles are spun in the usual way but are subjected during processing to different operations which serve to alter the physical characteristics of one or more, but not all, of the thread bundles. The application to the thread bundles of media designed to produce such effects as modified color, diminished luster, increased curliness, etc., is within the purview of this phase of the invention. One or several such operations may readily be accomplished by providing the appropriate number of reels in the series or, if desired, by employing two or more distributors 39 at existing positions in each series.

As has already been indicated, loosely aggregating several dissimilar thread bundles, cutting the resulting large thread bundle into chips, and subjecting the chips to a blending operation re-

sults in a uniform intermingling of the fibers lending itself to the production of novel effects when the product is ultimately spun into yarn. The commingling of straight and curly fibers, for instance, gives rise to such an effect. Substantially the same novel results that have already been described in connection with the first phase of the invention may also be obtained by means of colors applied externally to thread bundles.

10 For example, the process of blending fibers of two primary colors to form a product of a single secondary color may be accomplished by the application of two or more dyestuffs to the thread bundles. In such case, the thread bundles to be dyed are subjected to the action of dyestuffs applied by means of distributors 39. Although continuously advanced along the respective reels, the thread bundles remain on the reels long enough to become fully dyed before passing to 15 succeeding reels. After the dyeing operation, the dyed thread bundles are joined, reduced to fibers of staple length, dried, and blended as before.

A wide variety of novel effects may be produced by the practice of the present invention. As previously indicated, the inventive concept is 20 equally applicable to products manufactured according to any of the well-known processes, whether it be the casein, cellulose acetate, nitrocellulose, cuprammonium or viscose process; in fact, according to any process by which two or 25 more multiple filament thread bundles may be produced simultaneously. It is intended that the patent shall cover, by suitable expression in the appended claims, whatever features of patentable 30 novelty reside in the invention.

35 What is claimed is:

1. A method of manufacturing from artificial silk thread staple fiber adapted to be spun into a novel yarn comprising the steps of simultaneously producing a plurality of artificial silk threads of like origin and of substantially continuous length at least one of which is characterized by a uniform color throughout its 40 length which differs from that of the remaining threads; joining said threads to form a single composite thread bundle; reducing the thread bundle to fibers of staple length; and blending the resulting fibers in such fashion that the individual colors cooperate to produce a novel 45 effect.

2. The method of manufacturing from artificial silk thread of substantially continuous length staple fiber adapted to be spun into a novel yarn comprising the steps of preparing a 50 plurality of like spinning solutions at least one of which contains a substance capable of developing a color in the thread produced therefrom; simultaneously extruding each of said spinning solutions from a separate spinneret into a common coagulant, thereby forming a number of threads of like origin and of different colors; joining said threads to form a single composite thread bundle; reducing the thread bundle to fibers of staple length; and blending the resulting fibers in such fashion that the different colors thereof cooperate to produce a heterochromatic effect.

3. The method of manufacturing from artificial silk thread of substantially continuous length staple fiber adapted to be spun into a novel yarn comprising the steps of simultaneously extruding a plurality of multiple filament threads of like origin in a coagulant; subjecting each of said threads to a series of processing treatments during the course of which at least 70 75

one of said threads will acquire a color which differs from that of each of the remaining threads; joining said threads to form a single composite thread bundle; reducing the thread bundle to fibers of staple length; and blending the resulting fibers in such fashion that the different colors thereof cooperate to produce a heterochromatic effect.

4. A method of manufacturing from artificial silk thread of substantially continuous length staple fiber adapted to be spun into polychromatic yarn characterized by a monochromatic appearance comprising the steps of preparing a plurality of like spinning solutions each of which contains a substance capable of developing a different color; simultaneously extruding each of said spinning solutions from a separate spinneret into a common coagulant, thereby forming a number of differently colored threads of like origin; joining said threads to form a single multi-colored thread bundle; reducing the thread bundle to fibers of staple length; and blending the resulting fibers in such fashion that the individual colors are virtually indistinguishable, whereby the products have the appearance of a single color.

5. The method according to claim 2 in which the substance added to the spinning solution is one of a class of pigment colorants.

6. The method according to claim 2 in which the substance added to each of the several spinning solutions is one of a class of leuco base dyestuffs.

5 7. The method according to claim 2 in which the substance added to the spinning solution is a vat dye.

8. The method according to claim 3 in which a vat dye is applied to each of the several threads 10 during the processing treatment.

9. The method of manufacturing from artificial silk thread of substantially continuous length staple fiber adapted to be spun into a polychromatic yarn characterized by a monochromatic appearance comprising the steps of simultaneously forming by an extrusion process a plurality of threads of like origin and of at least two different colors; subjecting said threads 15 individually to each of a series of processing 20 treatments; joining said threads to form a single multi-colored thread bundle; cutting the thread bundle to fibers of staple length; drying the resulting staples and blending the same in such fashion that the individual colors are virtually 25 indistinguishable whereby the products have the appearance of a single color.

LOUIS S. FRYER.